

# UNITED STATES PATENT OFFICE.

WALTER BENTLEY WOODBURY, OF LONDON, ENGLAND, ASSIGNOR TO  
FREDERICK NEVILL CLARKE, OF SAME PLACE.

## PRODUCING GELATINOUS PRINTING-PLATES.

SPECIFICATION forming part of Letters Patent No. 310,486, dated January 6, 1885.

Application filed February 16, 1884. (No specimens.) Patented in Belgium November 14, 1879, No. 49,819, June 9, 1880, No. 51,708, and July 7, 1881, No. 55,113; in France November 15, 1879, No. 133,677, and in England June 10, 1881, No. 2,527.

*To all whom it may concern:*

Be it known that I, WALTER BENTLEY WOODBURY, of London, England, have invented a certain new and useful Method or 5 Process of Producing Photographic Gelatinous Printing-Plates; and I do hereby declare that the following specification is a clear, true, and complete description of my invention.

This invention has been patented in Europe 10 as follows, to wit: Great Britain, June 10, 1881, No. 2,527; addition dated March 26, 1880, to French Patent No. 133,677, November 15, 1879, and in two additions, June 9, 1880, No. 51,708 B, and July 7, 1881, No. 15 No. 55,113 B to Belgian Patent, November 14, 1879, No. 49,819 B.

A photographic gelatinous printing-plate produced by me in accordance with my invention is novel, in that the printing-surface 20 thereof is coated with metal foil, preferably tin-foil, and in some cases said plates are provided with a thin layer or film of caoutchouc interposed between the foil and the gelatinous matter, and in other cases I electroplate 25 the foil printing-surface; and it is to be understood that such photographic printing-plates are included, broadly, within the claims of my application for Letters Patent, Serial No. 103,326, and are specifically claimed in 30 my application, Serial No. 121,340, filed herewith, and bearing the Serial No. 121,340, as a division of my prior application No. 103,326. For producing these plates I proceed as follows: I prepare upon a plate of glass a gelatinous 35 printing-surface of any design or picture by means of light, as by the ordinary and well-known processes of photography, and upon said surface I place a sheet of metal foil, and over that a sufficient number of thicknesses of 40 blotting-paper or other soft-sheeted smooth-surfaced material, and then pass the whole through an ordinary roller-press, or apply sufficient pressure in any manner, so as to force or press the foil into intimate contact with 45 every part of the photographic design on the surface of the gelatine, and thereby develop on the surface of the foil every line and detail of said design.

When semi-transparent colors are to be employed in printing, as in what is known as the "Woodbury process," I prepare the gelati-

nous foil-coated plates from photographic foundations, as follows: I prepare a gelatinous compound composed, preferably, of, say, four hundred and fifty parts gelatine, water eighteen hundred parts, glycerine sixty parts, sugar forty-five parts, and a small quantity of liquid india-ink. Thin sheets of this compound are formed on plates of glass or other similarly-surfaced material, thoroughly dried, 55 and then stripped therefrom. When required for use, these sheets are sensitized by a bath of bichromate-of-potash solution of a strength of, say, six per cent., and properly dried. A sheet thus sensitized and mounted upon a solid 60 back is exposed to the light under a photographic "positive," (or a "negative," as the case may be,) and then developed in warm water, wherein the soluble parts are washed away in a manner well known, leaving the 70 photographic design in relief, whereupon the plate is washed with strong spirit, which absorbs the water from the gelatinous matter and speedily causes it to dry. When properly dried, the surface is coated with a thin 75 solution of caoutchouc in benzole or other suitable solvent, and thereon a sheet of tin-foil is laid and subjected to pressure, as before described, for developing the photographic design upon the surface of the foil, 80 which serves as the printing-surface. When said foil-coated photographic gelatinous printing-plates are to be relied upon for extensive printing service, I deposit upon the foil-surface, in a manner common to electroplating, a 85 layer of metal harder than the foil, such as copper or nickel.

Having thus described my invention, I claim as new and desire to secure by Letters Patent—

1. The method of producing photographic 90 gelatinous printing-plates by first developing a photographic design upon a sheet of gelatinous matter, then drying and mounting said sheet upon a solid back, and then coating the surface of said sheet with tin-foil applied 95 thereto under pressure, for developing on the surface of the foil the photographic design, and thereby affording a metallic printing-surface for reproducing said design, substantially as described.

2. The method of producing foil-coated photographic gelatinous printing-plates by ap-

plying between the foil and the gelatinous matter a thin layer or film of caoutchouc, and then subjecting the foil to pressure, substantially as described.

5 3. The method of producing photographic gelatinous printing-plates by first developing a photographic design upon a sheet of gelatinous matter, then coating said sheet with

foil and developing said design on the surface of said foil by pressure, and then electroplating said foil surface, substantially as described.

WALTER BENTLEY WOODBURY.

Witnesses:

HENRY J. FULLER,  
SAM. P. WILDING.